

## UNITED STATES PATENT OFFICE

J PEARL WILSON, OF JACKSONVILLE, FLORIDA, ASSIGNOR TO WILSON-OTWELL & CONE, INC., OF JACKSONVILLE, FLORIDA, A CORPORATION OF FLORIDA

## METHOD OF DRYING LUMBER

No Drawing.

Application filed October 6, 1927. Serial No. 224,528.

This invention relates to an improvement in a method of drying lumber.

The object of the invention is to dry lumber thoroughly to the center before the pores of the lumber have had an opportunity to close, and before shutting in the moisture and making it necessary to use sufficient heat or drying medium to open these pores before it is possible to withdraw the moisture. It has been found in practice that a large amount of heat is wasted in this way. It can be saved if the drying operation takes place before the pores of the lumber have closed.

When the lumber is sawed, the pores are open, and in the case of small lumber it may be run directly into the dry kiln where the drying may take place. It is however undesirable to mix the large and small lumber together, because the latter dries very much quicker than the former, and there should be a separation in order that the small lumber may be removed from the kiln when it is thoroughly dried, while allowing the large size to remain therein a sufficient length of time required to remove the moisture content.

In sawing a log, it is cut into several different pieces of varying sizes in order to obtain the greatest possible amount of lumber while decreasing the amount of waste. In order to do this, there will only be a small number of pieces of large size with a greater number of small size. The latter accumulate a great deal faster than the former, and since these should not be placed on the same truck for the drying operation but instead should be separated, it will take considerable time very often in which to accumulate a truck-load of the large size. In order that it will not have to remain in the open air during this time, which would tend to close its pores, it is preferable that this lumber should be immersed in hot water to keep the pores open and to heat it entirely to the center.

Therefore this invention involves the taking of the lumber directly from the saw and as soon as possible after the sawing operation, before the pores have had an opportunity to close, stacking it on a cradle with the usual sticks between the lumber and lowering this

cradle into a tank of hot water which, however, is not sufficiently hot, as to cause a scalding of a workman, and then raising the temperature of the water approximately to boiling point, namely 212 degrees F., in order to heat the lumber to its center and to prevent the closing of its pores. Whenever the lumber is thus heated throughout, it may be withdrawn from the tank of hot water and loaded on a truck and run directly into the dry kiln where it will dry along with the small sized lumber and in approximately the same length of time.

The cradle may be lowered into the tank by means of a hoist or other suitable arrangement. The heating of the water may be by means of steam or steam coils arranged in the tank sufficient for this purpose. The large sized lumber is placed on a cradle preferably as soon as it is taken from the saw, but at any rate before the pores have had an opportunity to close, and it is immediately lowered into the tank of hot water, and after a full charge has accumulated on this cradle the temperature of the water is raised to boiling point, as mentioned above. This heats the lumber throughout and entirely to the center without exposure to the air, after which it is ready to be placed in an ordinary dry kiln, which should be done without delay, where the heat of the kiln and the heat of the lumber cause a drying of the lumber from the center outwardly, instead of from the outside inwardly, and allows the pores to contract and the shrinkage to take place in an even, normal manner without injury to the lumber.

This method of drying is especially applicable to red gum, southern oak, and other kinds containing a large percentage of moisture content, because it allows for an even removing of the moisture without case-hardening and preventing inside honeycombing. The time required for the lumber to remain in its hot bath depends upon the kind and thickness of the lumber.

In this way a new method of drying lumber has been devised which has proven very successful, and it is a radical departure from the usual method of drying lumber, accom-

plishing a more thorough drying operation in a very much shorter length of time than where the lumber is allowed to stand in the air until after its pores are closed.

5 Reference in the claims to the closing of the pores of the lumber is intended to designate either a contraction of the cellular structure and, or, a sealing of the pores due to the resins, sap, etc., contained in the wood, which becomes oxidized to form a seal.

10 10 claim:—

1. A method of drying lumber including immersing the lumber in a hot bath before the pores have become closed.

15 2. A method of drying lumber including immersing the lumber in a hot water bath before the pores have had an opportunity to become closed.

20 3. A method of drying lumber including immersing the lumber in a hot water bath immediately after sawing and before the pores have had an opportunity to close, and thereafter subjecting the lumber to artificial drying.

25 4. A method of dry lumber including passing the lumber directly from the sawing operation into a hot water bath before the pores have had an opportunity to become closed, raising the temperature of the hot water bath 30 to approximately boiling point for heating the lumber to the center and thereafter directly subjecting the lumber to artificial drying for completing the drying operation.

35 5. A method of drying lumber including passing the lumber directly from the sawing operation into a hot water bath before the pores of the lumber have become closed, raising the temperature of the hot water bath approximately to boiling point, allowing the 40 lumber to remain in said hot water bath until heated approximately to its center and thereafter removing the lumber and subjecting the lumber to artificial drying for completing the drying operation and allowing an even 45 and thorough drying of the lumber.

In testimony whereof I affix my signature.  
J PEARL WILSON.